

## UNITED STATES PATENT OFFICE

ROBERT MARIA GERLACH, OF BERLIN-HALENSEE, GERMANY

## HEAVY METAL NAPTHENATE

No Drawing. Application filed June 21, 1926, Serial No. 117,596, and in Germany October 13, 1924.

This invention refers broadly to a new class of pigments, impregnating and similar compounds, and it is intended to devise means of producing a more generally applicable class of compounds of the kind referred to than it was generally possible to obtain by the processes heretofore in use. In the manufacture of pigments, staining, painting and impregnating compounds it is of importance 10 to provide means for the dissolving of heavy metal salts in oils, in order to thereby increase their preserving, bactericide and fungicide action. In view of the fact that metal salts are not soluble in tar oils, mineral oils and 15 fatty oils, as a general rule, solutions of such metal salts could be obtained heretofore almost exclusively by the assistance of soaps, by which means the metal salts were incorporated in the oils.

20 It has now been ascertained, in accordance with this invention that free fatty acids as well as free naphthenic acids and abietinic acids are adapted to produce complex compounds with heavy metal salts which are 25 soluble in oils, so that they are adapted to be dissolved in any proportions in tar oils, mineral oils, tar oils from lignite or brown-coal, peat-tar-oils or fatty oils and the like, by proceeding for instance in the following 30 manner:

*Examples:*—1. 100 parts by weight of American resin which is known to consists of about 75% abietic acid, are dissolved in 100 parts by weight of gas oil and are digested in a mixture with 3 parts by weight of copper-formiate, until a complete solution is obtained.

2. 100 parts by weight of naphthenic acid is heated with 6 parts by weight acetate of lead, until complete solution is obtained.

3. 100 parts by weight of oleic acid is shaken up with a saturated aqueous solution of silico-fluorate of copper and the resultant precipitate is separated from the remaining aqueous liquid.

The complex compounds thus produced of the fatty acids, naphthenic acid, of the abietic acid and of the ferro-cyanic and ferri-cyanic acids may be used alone or in admixture with

oils, varnishes, japans or pigments for painting or for impregnating purposes and for similar uses.

Having thus described my invention and a number of exemplifications thereof it is 55 pointed out that the invention is not restricted to these particular exemplifications and mode of operation, but it is susceptible of modifications and changes within the scope and spirit of the invention as more particularly set forth 60 and pointed out in the appended claims.

All metals belonging to the so-called sulphuretted hydrogen group are adapted to be used in connection with the present invention and the metals mentioned in the foregoing, 65 namely, copper, lead and mercury, belong to that group. The expression "metals of the sulphuretted hydrogen group" comprises all metals which are precipitable in an acid solution with sulphuretted hydrogen. 70

I claim:

1. A process of manufacturing water-insoluble complex metal compounds, consisting in mixing 100 parts by weight of naphthenic acid with 6 parts by weight of acetate 75 of lead at ordinary temperature and digesting the mixture until complete solution is obtained.

2. A process of manufacturing water-insoluble complex metal compounds, consisting 80 in mixing naphthenic acid at ordinary temperature with acetate of lead and digesting the mixture until complete solution is obtained.

3. A process of manufacturing water-insoluble complex metal compounds, consisting in mixing naphthenic acid at ordinary temperature with salts of metals of the second analytical group with weak acids and digesting the mixture until complete solution is obtained. 85

In testimony whereof I affix my signature.

ROBERT MARIA GERLACH.